

## UNITED STATES PATENT OFFICE

OLIVER W. STOREY, OF MADISON, WISCONSIN, ASSIGNOR TO BURGESS BATTERY COMPANY, OF MADISON, WISCONSIN, A CORPORATION OF WISCONSIN

## PRODUCTION OF MANGANESE DIOXIDE

No Drawing.

Application filed May 12, 1931. Serial No. 536,937.

This invention relates to the production of manganese dioxide by an electrolytic method and more particularly to its production from rhodochrosite, a manganese carbonate ore, by a cyclic process.

It is an object of this invention to provide a simple, efficient, cyclical process for producing high grade electrolytic manganese dioxide from manganese carbonate ore. It is a further object to provide an improved electrolyte for the electrolysis operation.

Rhodochrosite, a manganese carbonate ore, is available in large quantities in Montana but it can not be changed directly by any known process into a suitable form of high grade manganese oxide since it is necessary to remove the impurities which are associated with it. These impurities usually are silica, calcite, magnesium carbonate, other silicious compounds and heavy metal compounds. If the manganese dioxide is to be used as a depolarizer in dry cells it is essential to remove these heavy metals since the presence of some of them in the depolarizer even in minute quantities would cause rapid deterioration of such cells.

I have discovered that it is possible to dissolve the Montana rhodochrosite ore in dilute sulphuric acid to form a solution containing manganese sulphate, then purify the resulting sulphate solution, and then electrolyze this purified solution to form manganese dioxide and dilute sulphuric acid. This sulphuric acid can be used to treat further quantities of the ore. The process thereby becomes cyclic with the simultaneous production of a high grade of manganese dioxide. It is therefore only necessary to supply as raw material in addition to the ore small amounts of sulphuric acid, to make up the losses in the process, and purification materials. All of the impurities present in appreciable amounts except the magnesium salts may be removed during the purification operations. The magnesium sulphate formed by the sulphuric acid, accumulates in the electrolyte. It is desirable, however, to have this salt present in the electrolyte and it is therefore not necessary to make any provision for its removal.

In carrying out my invention the man-

ganese carbonate ore is ground to a powder, preferably to about 100 mesh or finer, to facilitate reaction with the dilute sulphuric acid that is employed to convert the carbonate to manganese sulphate. It is preferable to use an ore that has a low calcite content since the sulphuric acid consumed in dissolving it is wasted, as the resulting insoluble calcium sulphate is discarded. The reaction is preferably carried out at near the boiling point of water in a counter-current system so that the insoluble portion of the ore which is discarded contains a minimum of undissolved manganese compounds. The resulting manganese sulphate solution is practically neutral.

The acid strength of the leaching liquor should be such that the resulting neutral solution preferably contains from 12% to 20% of manganese sulphate. With greater concentrations the solution becomes more difficult to handle, its purification becomes more difficult, and there is a decrease in the rate of solution of the manganese carbonate. Obviously the solution preferably should not be more dilute than the minimum strength used in the electrolytic cells. The dilute acid coming from the electrolytic cells after electrolysis contains manganese sulphate since the manganese is not completely removed. Sufficient sulphuric acid is added to this depleted electrolyte to make up for mechanical losses and losses due to the formation of sulphates other than manganese, due to the presence of impurities in the ore as previously described. Except for the addition of sulphuric acid to cover these losses, the depleted electrolyte contains the correct amount of sulphuric acid to secure the desired manganese sulphate concentration in the leaching operation.

The manganese sulphate solution is decanted or filtered from the insoluble of the ore. The hot solution is then oxidized, preferably by aeration. A regulated amount of finely divided calcium carbonate is employed during oxidation to neutralize the acid formed by the hydrolysis of ferric sulphate. The iron is thereby completely precipitated as ferric hydrate. The electrolyte should be free from iron as small quantities

of it will greatly decrease the current efficiency. Magnesium carbonate or manganese carbonate may also be used to maintain the neutrality of the solution. The hydrates or oxides may be used instead of the carbonates, but these substances tend to precipitate the manganese as a hydrate, which is oxidized readily to brown oxides. The manganese sulphate solution is filtered and is ready to be used in the electrolytic cells after being diluted to the desired concentration. The solution should not contain any or only minute amounts of any compounds which will cause reduction of the manganese dioxide formed during electrolysis. Ferrous compounds and certain organic materials are examples of these reducing compounds.

The electrolysis is preferably carried out in a hot solution along the lines described by Van Arsdale and Maier (see Patent No. 1,304,222 and Trans. Am. Electrochem. Soc., Vol. 33, p. 109, 1918) but modified for cyclical operation. Lead lined tanks may be used, the lead preferably being hardened. The anodes may be platinum or graphite, the latter being impregnated with bakelite or similar water and acid resisting material to prevent rapid disintegration. I prefer, however, to use lead which has been hardened to prevent sagging which occurs in the hot electrolyte when pure lead is used. The hardened anode also facilitates the removal of the manganese dioxide deposit. Lead hardened with about 6% of antimony has given good results. The percentage of antimony may be varied. Various lead alloys such as lead-silver, lead-thallium and others may be used. The cathode may be of graphite or suitable metals or alloys. The electrolyte should be kept hot, 90° C. being a favorable temperature. A current density of about 6 to 10 amperes per square foot gives good results. Good results have been obtained with an electrolyte containing about molar manganese sulphate, or the equivalent mixture of manganese sulphate and sulphuric acid. Under the above conditions of electrolysis the current efficiency is not decreased by the replacement of the manganese sulphate by its equivalence in sulphuric acid until the manganese sulphate content drops below about  $\frac{1}{3}$  molar. The electrolysis may therefore be conducted at the highest efficiency under wide limits of sulphuric acid and manganese sulphate ratios. It is desirable theoretically for the electrolyte to contain as high a content of manganese sulphate or equivalent mixture with sulphuric acid as possible but practical considerations interfere with the use of saturated or nearly saturated solutions. I have found that an electrolyte containing about 150 grams  $MnSO_4$  per liter gives excellent results though concentrations of 100 grams to 200 grams per liter may be used. These concen-

trations include the sulphuric acid present in terms of equivalent manganese sulphate. Above 200 grams per liter the solution becomes too heavy and various difficulties are encountered at certain points in the process.

Instead of electrolyzing the purified neutral manganese sulphate solution under the above conditions until the manganese content is practically exhausted to produce dilute sulphuric acid as a by-product as has heretofore been done, this solution is fed into the electrolytic cell continuously at a predetermined rate proportionate to the current. There is withdrawn at another point, a like amount of exhausted electrolyte which contains for example, 30 grams manganese sulphate per liter and 78 grams sulphuric acid per liter, thereby making the deposition continuous in contrast to the above mentioned intermittent process. This exhausted electrolyte is then returned to the first step in the process to be used in the treatment of manganese carbonate ore. Since the electrolysis may be carried out with equal efficiency in electrolytes containing smaller amounts of manganese sulphate and larger amounts of free acid as previously explained, I prefer to recirculate a large proportion of the exhausted high-acid electrolyte with the incoming neutral sulphate electrolyte so that the electrolysis is conducted with an electrolyte that is practically of uniformly high acid content throughout the cell. Better electrolyte circulation is also secured by this method. In a specific example the incoming neutral electrolyte (taken as one volume) contains 150 grams manganese sulphate per liter and the exhausted electrolyte contains 50 grams manganese sulphate and 66 grams sulphuric acid per liter. Exhausted electrolyte equal in volume to the neutral electrolyte is returned to the leaching operation to react with the ore. However, an additional three volumes of exhausted electrolyte are withdrawn at the same time and mixed with the incoming neutral electrolyte so that the incoming electrolyte (a mixture of one volume of neutral and three volumes exhausted) is composed of 75 grams manganese sulphate and 49 grams sulphuric acid per liter. These proportions are merely illustrative and may vary over a wide range to suit the specific conditions.

The manganese dioxide, which is deposited at the anode, is readily detached therefrom, after which it is washed free of sulphates and sulphuric acid. By using the above methods manganese dioxide has been electrodeposited without difficulty to a thickness of over one inch.

It has been found further that when magnesium sulphate is present in the manganese sulphate electrolyte the power efficiency of electrodeposition (hot electrolyte) is increased considerably. This increased effi-

ciency apparently results mostly or entirely from the decrease in impressed voltage on the cells. My measurements show that the impressed voltage is decreased from 15% to 5 30% when magnesium sulphate is added to a hot, pure, neutral manganese sulphate electrolyte. As low as 0.1% of magnesium sulphate has a marked effect. I prefer having at least 2% of magnesium sulphate in the 10 electrolyte. Excellent results have been obtained with an electrolyte containing about 8% to 12% of magnesium sulphate. Higher percentages may be used. Under the conditions of continuous operation described it 15 was found that with a rhodochrosite containing 3.15% magnesium carbonate, the electrolyte seldom contained more than about 10% of magnesium sulphate, probably because of certain unknown equilibrium conditions, al- 20 though it is possible to dissolve considerably more than this amount of magnesium sulphate in pure manganese sulphate solutions of equal strength. Such solutions containing in excess of 10% of magnesium sulphate 25 may be electrolyzed to produce manganese dioxide with excellent result.

The manganese carbonate ore usually contains magnesium carbonate, which dissolves in the sulphuric acid of the leaching solution to form magnesium sulphate. There may be more than sufficient carbonate in the ore to maintain the desired amount of the magnesium sulphate in the electrolyte without the extraneous addition of this salt. Because of the probable equilibrium conditions mentioned above the electrolyte does not seem to accumulate an excess of magnesium sulphate where there is not an excessive amount of magnesium carbonate in the ore. 40 It, therefore, does not become necessary to discard the electrolyte from time to time because of the accumulation of too much magnesium sulphate in it, with the consequent loss of manganese sulphate and sulphuric acid which would be entailed.

I claim:

1. A solution for use in the production of electrolytic manganese dioxide which comprises a water solution of neutral purified manganese sulphate containing magnesium sulphate in an amount sufficient to depress markedly the impressed voltage required for the hot electrolysis of said solution to produce said dioxide.
2. A solution for use in the production of electrolytic manganese dioxide which comprises a water solution of purified manganese sulphate, said solution containing at least 100 grams per liter of said sulphate and at least 0.1% magnesium sulphate.
3. An electrolyte for the production of electrolytic manganese dioxide which comprises a water solution of purified manganese sulphate, said solution containing at least 100 grams per liter of combined manganese sul-

phate and sulphuric acid in terms of equivalent manganese sulphate, but not less than about 30 grams per liter of said sulphate, and at least 2% magnesium sulphate.

4. A solution for use in the production of electrolytic manganese dioxide which comprises a water solution of purified manganese sulphate, said solution containing from about 100 grams to 200 grams per liter of said sulphate, and at least 2% of magnesium sul- 70 phate. 75

5. An electrolyte for the production of electrolytic manganese dioxide which comprises a water solution of substantially iron-free manganese sulphate, said solution containing from 100 grams to 200 grams per liter of combined manganese sulphate and sulphuric acid in terms of equivalent manganese sulphate, but not less than about 30 grams per liter of said sulphate, and at least 2% of magnesium sulphate. 80

6. The method for appreciably depressing the voltage impressed on a hot manganese sulphate solution to produce manganese dioxide therefrom, which comprises introducing about 0.1% or more of magnesium sulphate into said electrolyte. 90

7. In the electrolytic production of manganese dioxide the method which comprises electrolyzing a purified hot manganese sulphate solution containing at least 100 grams per liter of combined manganese sulphate and sulphuric acid in terms of manganese sulphate, but not less than about 30 grams per liter of said sulphate, and at least 2% of 95 magnesium sulphate. 100

8. In the electrolytic production of manganese dioxide the method which comprises electrolyzing a purified hot manganese sulphate solution containing from 100 grams to 200 grams per liter of combined manganese sulphate and sulphuric acid in terms of manganese sulphate but not less than about 30 grams per liter of said sulphate, and at least 0.1% of magnesium sulphate. 110

9. In the electrolytic production of manganese dioxide the method which comprises electrolyzing with a cathode and a hardened lead anode a substantially iron-free hot manganese sulphate solution containing from 100 grams to 200 grams per liter of combined manganese sulphate and sulphuric acid in terms of manganese sulphate but not less than about 30 grams per liter of said sulphate, and at least 2% of magnesium sulphate. 115

10. In the cyclical process of continuous electrolytic production of manganese dioxide the method which comprises adding continuously a purified manganese sulphate solution containing magnesium sulphate to the electrolyte to replenish the manganese sulphate content and withdrawing continuously an equivalent amount of depleted electrolyte containing magnesium sulphate. 120

11. In the cyclical process of continuous 125

electrolytic production of manganese dioxide  
the method which comprises adding continuously a purified and substantially iron-free  
hot manganese sulphate solution containing  
from 100 grams to 200 grams per liter of  
manganese sulphate and at least 0.1% of  
magnesium sulphate to the electrolyte to re-  
plenish the manganese sulphate content and  
10 withdrawing continuously an equivalent  
amount of depleted electrolyte containing  
magnesium sulphate.

In testimony whereof I affix my signature.  
**OLIVER W. STOREY.**

**15****20****25****30****35****40****45****50****55****60****65**